

# United States Patent Office

3,000,895

Patented Sept. 19, 1961

1

3,000,895

## POLYNITROPIPERIDINES

Milton B. Frankel, Pasadena, Calif., assignor to Aerojet-General Corporation, Azusa, Calif., a corporation of Ohio

No Drawing. Filed Oct. 3, 1957, Ser. No. 688,808  
11 Claims. (Cl. 260—293)

This invention relates to new compositions of matter and to their preparation. In particular, the invention relates to polynitropiperidines having the general formula:



wherein R and R' are hydrogen or nitro radicals.

This application is a continuation-in-part of my copending U.S. application Serial No. 392,473, filed November 16, 1953, now abandoned.

The polynitropiperidines of this invention, such as 3,3,5,5-tetranitropiperidine, condense with nitro alcohols, such as trinitroethanol, to form high explosive compounds such as N - (2,2,2 - trinitroethyl) - 3,3,5,5 - tetranitropiperidine, as more fully disclosed in my copending U.S. application Serial No. 628,949, filed December 12, 1956. Also, the compounds of this invention, such as 3,3,5,5-tetranitropiperidine, react with nitric acid to form explosive compounds such as N-3,3,5,5-pentanitropiperidine, as more fully disclosed in my copending U.S. application Serial No. 617,668, filed June 25, 1957.

The compounds formed from the polynitropiperidines of the present invention, as taught in the above-mentioned U.S. applications Serial No. 628,949 and Serial No. 617,668, are useful as high explosives and can be used in any conventional explosive missile, projectile, rocket, or the like, as the main explosive charge. An example of such a missile is disclosed in United States Patent No. 2,470,162 issued May 17, 1949. One way of using these high explosive compounds in a device such as that disclosed in United States Patent No. 2,470,162 is to pack the crystalline explosive in powder form into the warhead of the missile. Alternatively, the crystals can be first pelletized and then packed. A charge thus prepared is sufficiently insensitive to withstand the shock entailed in the ejection of a shell from a gun barrel or from a rocket launching tube under the pressure developed from ignition of a propellant charge, and can be caused to explode on operation of an impact- or time-fuse mechanism firing a detonating explosive such as lead azide or mercury fulminate.

The polynitropiperidines of this invention are prepared by condensing ammonium salts of carboxylic acids with polynitro-1,5-pentanediol, in accordance with the general reaction scheme set forth below:



wherein R and R' are as defined above and R'' is a lower alkyl radical.

To more clearly illustrate my invention, the following example is presented. It is to be understood, however, that this example is intended merely as an illustrative em-

2

bodiment of the invention and it should not be construed as limitative of the scope of said invention in any way.

### EXAMPLE

#### Preparation of 3,3,5,5-tetranitropiperidine

In a 125-ml. Erlenmeyer flask was placed a solution of 4 gm. (0.052 ml.) of ammonium acetate in 40 ml. of water and 4 gm. (0.014 ml.) of 2,2,4,4-tetranitro-1,5-pentanediol. The solution was warmed to 40–50° C. and after several minutes an orange solid separated. The solid was collected and dried to give 2.0 gm. (53.7%) of 3,3,5,5-tetranitropiperidine, M.P. 108–112° C. Recrystallization from isopropyl alcohol gave white needles M.P. 123–127° C.

15 *Analysis.*—Calc'd for  $C_5H_5N_5O_8$ : percent C, 22.65; percent H, 2.66; percent N, 26.42. Found: percent C, 23.46; percent H, 2.94; percent N, 26.61.

The polynitro-1,5-pentanediol starting materials for the reaction of this invention, such as the 2,2,4,4-tetra-1,5-pentanediol of the above example, are readily obtained by reacting an alkali metal or alkaline earth metal salt of polynitrobutanol, such as potassium 2,2,4,4-tetranitrobutanol, with formaldehyde, as more fully disclosed in assignee's copending U.S. application Serial No. 662,550, filed May 29, 1957.

20 It is preferred, for reasons of convenience, to conduct the reaction of this invention in an aqueous solution. I have found that optimum results are obtained in the practice of my invention, when an aqueous medium is employed, when the reaction temperature is within the range from about 25° to about 50° C., although higher or lower reaction temperatures can be employed within the scope of my invention.

25 It will be appreciated that any of the polynitropiperidines within the scope of my invention can be prepared by the method taught herein. For example, 2,4-dinitro-1,5-pentanediol and 2,2,4-trinitro-1,5-pentanediol condense with ammonium salts of lower carboxylic acids, such as ammonium formate, ammonium butyrate etc., to yield 3,5-dinitropiperidine and 3,3,5-trinitropiperidine, respectively.

30 I claim:

1. As compositions of matter, the polynitropiperidines having the formula:



35 wherein R and R' are radicals selected from the group consisting of hydrogen and nitro radicals.

2. As a composition of matter, 3,3,5,5-tetranitropiperidine having the structural formula:



40 3. As a composition of matter, 3,5-dinitropiperidine.

4. As a composition of matter, 3,3,5-trinitropiperidine.

45 5. The method of preparing polynitropiperidines having the formula:



which comprises condensing a polynitro-1,5-pentanediol having the formula:



with the ammonium salt of a carboxylic acid having the formula:



10

wherein R and R' are radicals selected from the group consisting of hydrogen and nitro radicals and R'' is a lower alkyl radical.

6. The method of preparing polynitropiperidines having the formula:



which comprises condensing a polynitro-1,5-pentanediol having the formula:



with the ammonium salt of a carboxylic acid having the formula:



wherein R and R' are radicals selected from the group

25

30

35

consisting of hydrogen and nitro radicals and R'' is a lower alkyl radical, at a temperature of from about 40° to about 50° C.

7. The method of preparing 3,3,5,5-tetranitropiperidine which comprises condensing 2,2,4,4-tetranitro-1,5-pentanediol with the ammonium salt of a carboxylic acid having the formula:



wherein R'' is a lower alkyl radical.

8. The method of preparing 3,3,5,5-tetranitropiperidine which comprises condensing 2,2,4,4-tetranitro-1,5-pentanediol with ammonium acetate.

9. The method of preparing 3,3,5,5-tetranitropiperidine which comprises condensing 2,2,4,4-tetranitro-1,5-pentanediol with ammonium acetate at a temperature of from about 40° to about 50° C.

10. The method of preparing 3,5-dinitropiperidine which comprises condensing 2,4-dinitro-1,5-pentanediol with the ammonium salt of a carboxylic acid having the formula:



wherein R'' is a lower alkyl radical.

11. The method of preparing 3,3,5-trinitropiperidine which comprises condensing 2,2,4-trinitro-1,5-pentanediol with the ammonium salt of a carboxylic acid having the formula:



wherein R'' is a lower alkyl radical.

No references cited.